

March 11, 1941.

J. J. KEYES

2,234,560

COVERED WIRE

Filed Nov. 16, 1938

Fig. 1.



Fig. 2.



Fig. 3.



Fig. 4.



WITNESSES:

*C. J. Weller*  
*James H. Ely*

INVENTOR

*John J. Keyes.*

BY

*Frank Savage*

ATTORNEY

## UNITED STATES PATENT OFFICE

2,234,560

## COVERED WIRE

John J. Keyes, Edgewood, Pa., assignor to Westinghouse Electric & Manufacturing Company, East Pittsburgh, Pa., a corporation of Pennsylvania

Application November 16, 1938, Serial No. 240,701

8 Claims. (Cl. 174—121)

This invention relates to wire having a covering of fibrous material.

Heretofore, electrical conductors have been produced having many different types of insulating coverings. In most of these cases it has been necessary to employ coverings containing organic material or which were not resistant to high operating temperatures.

An object of this invention is to provide a wire having an inorganic covering.

Another object of this invention is to provide a wire having a covering of inorganic material disposed about the wire in different forms whereby each form functions to best advantage in maintaining the wire completely insulated.

A more specific object of this invention is to utilize glass fibers of both the staple and continuous filament types as the covering for wire, the staple type fibers being adjacent the wire and providing a cushion or yielding layer for the continuous filament type of fibers to facilitate the making and maintenance of a completely insulated conductor under operating conditions.

A further object of this invention is to provide a wire having a covering formed from substantially alkaline-free glass fibers of the staple and continuous filament types applied thereto in a predetermined manner and coated and impregnated with an insulating varnish.

Other objects of this invention will become apparent from the following description when taken in conjunction with the accompanying drawing, in which

Figure 1 is an elevational view, greatly exaggerated, of a covered wire embodying this invention;

Fig. 2 is a sectional view taken along the line II—II of Fig. 1;

Fig. 3 is an elevational view of another embodiment of this invention; and

Fig. 4 is a sectional view taken along the line IV—IV of Fig. 3.

Referring to Figs. 1 and 2 of the drawing, this invention is illustrated as embodying the wire 10 covered with an inorganic material. The inorganic material employed as the covering is formed from glass fibers which are nonhygroscopic and, as compared to asbestos and other materials employed heretofore, have no metallic particles, higher dielectric strength, lower insulation losses, better heat conductivity, better space factor and are more uniform in coverage and thickness.

In accordance with the invention, the covering

of inorganic material on the wire is formed from a plurality of layers of material having the same composition but which are in different form. The preferred inorganic material utilized is glass formed into very fine fibers. It has only recently 5 been commercially possible to spin the glass into fibers sufficiently fine to permit their use as embodied in this invention. These fibers have a diameter of .00025 inch or less and in this state are not as brittle as the heavier fibers. 10

In manufacturing the glass fibers utilized in this invention, two processes are now generally employed. These are known as the continuous filament process and the staple fiber process. In the continuous filament process, glass of predetermined composition is melted and continuous filaments, usually 102 in number, are drawn from the melt onto a spool after which the filaments are worked into yarns, tapes, etc., in a manner similar to the making of rayon. As distinguished 20 from the continuous filament process, the staple fibers are produced from the molten glass by drawing them from the melt by means of a blast of steam applied to the glass as it leaves the reservoir, thereby breaking the glass into fine fibers 25 of different length. As a general rule, the staple fibers are not over from 10 to 12 inches in length, the average being about 6 to 8 inches. The staple fibers may be worked into yarn in a manner similar to the process in making cotton yarn. 30

The glass which it is preferred to utilize in this invention is one which is substantially alkaline-free, containing not over 5% of soda. If a higher soda content is present, the glass has poor stability under changing humidity conditions, the moisture encountered drawing the alkali from the glass and causing the fibers to quickly deteriorate. This poor stability of the higher alkaline glass can, however, be overcome if an impregnating material which contains a weak organic acid is employed in conjunction with the glass, the weak organic acid functioning to neutralize the alkalinity of the glass. 35

In covering the wire 10, a layer 12 of the unwoven staple fibers is formed around and over the wire in thread or yarn form. This layer may also be felted or spun on to the wire direct from the glass reservoir or furnace or in a manner comparable to the known methods of applying asbestos to wire, as in the form of roving. As formed around the wire, the layer 12 is soft and fluffy having a certain amount of resiliency under shock. These staple fibers are, however, not satisfactory as a finished covering on the wire 50 55

since they do not have the desired strength and resistance to abrasion. Further, since the fibers are relatively short, the surface of the layers 12 has a very fuzzy appearance because of the ends 5 of the fibers projecting therefrom.

In order to provide a smooth finish to the conductor covered with the staple fibers, and to provide increased resistance to abrasion, a layer 14 of the glass fibers of the continuous filament type 10 is employed. This type has the strength necessary for maintaining itself as an integral covering and when applied around the layer of staple fibers covers the loose fuzzy ends. The covering of the continuous filament fibers may be 15 formed either by helically winding the yarn directly over the staple fibers or by applying the continuous filament fibers thereto in the form of tape, braid, sleaving or any other suitable form.

The two layers of glass fibers in different forms 20 cooperate with each other in giving a highly desirable article. Since the layer of the staple fiber is somewhat resilient, it acts as a cushion or yielding layer for the continuous filament layer which is inherently more brittle in bulk than the staple 25 fiber, permitting bending of the covered wire without damage to the outer covering. In service it is found that the layer of staple fibers prevents the breaking or cutting of the outer layer formed from the continuous filaments by abrasion or 30 pounding when the covered wire is employed in industry. Because the outer covering is of the continuous filament, it gives a covering of high strength which has a very smooth appearance and functions to retain the comparatively short 35 staple fibers of the inner layer in position about the wire. Both the staple fibers and the continuous fibers are inorganic materials which have an exceedingly high dielectric strength and high heat conductivity and which, because of their size, 40 may be utilized as very thin layers over the wire.

In service it is sometimes desirable to utilize 45 an impregnating compound or varnish in conjunction with the inorganic glass fiber coverings of this invention. Different types of impregnating compounds may be utilized depending upon the types of service in which it is desired to employ the covered wire. Suitable impregnating compounds or varnishes are those known to the trade 50 as oxidizing oil varnishes, oleoresinous varnishes or the impregnating insulating heat reactive types, such as the phenol formaldehyde and alkyd type resins or vinyl acetate. The use of such an impregnating compound or varnish is illustrated in 55 Figs. 3 and 4 in which 16 indicates a layer of the impregnating material formed on the covering of the continuous filament fibers, it being understood that this impregnating material penetrates the interstices of the glass fibers of both the inner 60 and outer layers forming the glass covering. The oxidizing oil and oleoresinous varnishes are to be preferred where the glass has a content of up to 5% of soda, since they will form weak organic acids to neutralize the small amount of alkali which may be encountered with such glass. 65 Where an impregnating material is used, it is preferred that the impregnated and covered conductor be subjected to sufficient heat to so fix or set the impregnating material that it is substantially stable under normal operating conditions. 70

Although this invention has been described with reference to a particular embodiment thereof, it is, of course, not to be limited thereto except insofar as is necessitated by the prior art and the 75 scope of the appended claims.

I claim as my invention:

1. An article of manufacture comprising a wire and a covering therefor, said covering comprising an inner resilient layer of unwoven substantially alkaline-free glass fibers of the staple type applied directly around and over the wire and an outer layer of substantially alkaline-free glass fibers of the continuous type, said outer layer being in the form of a braid of the continuous fibers and being applied directly around and over the inner 5 resilient layer of glass fibers.

2. An article of manufacture comprising a wire and a covering therefor, said covering comprising an inner layer of unwoven substantially alkaline-free glass fibers of the staple type adjacent the wire and an outer layer of substantially alkaline-free glass fibers of the continuous type, the layer of unwoven glass fibers forming a resilient backing for the outer layer, and a coating of insulating varnish on the outer layer of glass fibers, the insulating varnish impregnating the inner and outer layers of glass fibers of different types. 15 20

3. An article of manufacture comprising a wire and a covering therefor, said covering comprising an inner resilient layer of unwoven substantially alkaline-free glass fibers of the staple type applied directly around and over the wire and an outer layer of substantially alkaline-free glass fibers of the continuous type, said outer layer being in the form of a braid of the continuous fibers 25 and being applied directly around and over the inner resilient layer of glass fibers, and a coating of insulating varnish on the outer layer of glass fibers, the insulating varnish impregnating the different inner and outer layers of glass fibers. 30 35

4. An article of manufacture comprising a wire and a covering therefor, said covering comprising an inner layer of unwoven substantially alkaline-free glass fibers of the staple type applied directly around and over the wire and an outer layer of substantially alkaline-free glass fibers of the continuous type applied directly over and around the inner layer, the fibers of the inner and outer layers having an average diameter of not more than .00025 inch, the inner layer of staple fibers being 40 sufficiently resilient to permit bending of the covered wire without damage to the outer covering. 45

5. An article of manufacture comprising a wire and a covering therefor, said covering comprising an inner layer of unwoven substantially alkaline-free glass fibers of the staple type applied directly around and over the wire and an outer layer of substantially alkaline-free glass fibers of the continuous type applied directly around and over the inner layer, the outer layer being in the form of yarn helically wound about the unwoven staple fibers of the inner layer for retaining them in 55 position about the wire.

6. An article of manufacture comprising a wire and a covering therefor, said covering comprising an inner layer of unwoven substantially alkaline-free glass fibers of the staple type applied directly around and over the wire and an outer layer of substantially alkaline-free glass fibers of the continuous type applied directly around and over the inner layer, the outer layer being in the form of yarn helically wound about the unwoven staple fibers of the inner layer for retaining them in 65 position about the wire, and an electrically insulating material associated with and disposed to fill the interstices of the fibrous layers. 70

7. An article of manufacture comprising a wire and a covering therefor, said covering comprising an inner layer of unwoven substantially alkaline- 75

free glass fibers of the staple type adjacent the wire and an outer layer of substantially alkaline-free glass fibers of the continuous type, the layer of unwoven glass fibers forming a resilient backing for the outer layer.

8. An article of manufacture comprising a conductor and a covering therefor, said covering comprising an inner layer of unwoven glass fibers of the staple type adjacent the wire and an outer 10 layer of glass fibers of the continuous type, the

layer of unwoven glass fibers forming a resilient backing for the outer layer, the glass fibers of each of the inner and outer layers containing not more than 5% of soda thereby being substantially alkaline-free, and a coating of insulating varnish on 5 the outer layer of glass fibers, the insulating varnish being an oleoresinous varnish and impregnating the inner and outer layers of glass fibers of different types.

JOHN J. KEYES. 10

## DISCLAIMER

2,234,560.—*John J. Keyes*, Edgewood, Pa. COVERED WIRE. Patent dated March 11, 1941. Disclaimer filed January 20, 1945, by the assignee, *Westinghouse Electric & Manufacturing Company*.

Hereby enters this disclaimer to claims 2, 4, and 7 of said patent.  
[*Official Gazette February 20, 1955.*]